

# United States Patent [19]

Balland

[11] 3,854,872

[45] Dec. 17, 1974

[54] **PROCESS FOR DYEING OF POLYACRYLONITRILE FIBERS**

[75] Inventor: **Jean Balland**, Chateaurenault, France

[73] Assignee: **Societe dite: Manufacture de Produits Chimiques PROTEX Societe Francaise a Responsabilite Limitee Siege, Paris, France**

[22] Filed: **Mar. 29, 1973**

[21] Appl. No.: **345,850**

[30] **Foreign Application Priority Data**

Apr. 7, 1972 France ..... 72.12861

[52] U.S. Cl. .... **8/169**, 8/177 R, 8/172

[51] Int. Cl. .... **D06p 5/06**

[58] **Field of Search**..... 8/169, 85, 172, 177 R

[56]

## References Cited

### UNITED STATES PATENTS

|           |         |                      |       |
|-----------|---------|----------------------|-------|
| 3,619,121 | 11/1971 | Boehmke .....        | 8/169 |
| 3,716,329 | 2/1973  | Komninos et al. .... | 8/169 |
| 3,773,463 | 11/1973 | Cohen et al. ....    | 8/169 |
| 3,785,768 | 1/1974  | Walz et al. ....     | 8/84  |

*Primary Examiner*—Benjamin R. Padgett

*Assistant Examiner*—B. Hunt

*Attorney, Agent, or Firm*—Browdy & Neimark

[57]

## ABSTRACT

A process for dyeing polyacrylonitrile fibers in an aqueous bath containing a cationic dye which utilizes as a retarding and equalizing agent 0.2-5 percent of a quaternized polyamino amide obtained by condensation of a fatty diacid and a polyamine followed by quaternization by a salt of epoxy propyltrialkyl ammonium.

**4 Claims, No Drawings**

### PROCESS FOR DYEING OF POLYACRYLONITRILE FIBERS

The present invention relates to the dyeing of polyacrylonitrile fibers with cationic dyes.

It is known that polyacrylonitrile fibers are dyed in general utilizing cationic dyes such as those for example of the series of triaryl methane, oxazine, etc.

The use of these dyes in general permits obtaining polyacrylonitrile fibers of brilliant and intense colors having good general strengths.

The application of cationic dyes onto the polyacrylonitrile fibers can be accomplished by different dyeing processes. However, in the bath dyeing, that is by exhausting dye baths, the taking up and the fixation of the dye into the fiber can be correctly obtained only at temperatures less than those in the vicinity of the boiling point of water.

It is known that at these temperatures, and generally starting at 80°C, the exhaustion of the cationic dye baths by the polyacrylonitrile fiber is produced too rapidly. The result of this rapid exhaustion of the dye baths is manifested frequently in practice according to the intensity of the colors obtained, by a lack of uniformity of the color of the material. It is for this latter reason that the dyeing of polyacrylonitrile fibers often necessitates the use of a retarding agent so as to restrain the speed of taking up of the dyes by the fiber and to obtain better uniformity.

The present invention more particularly relates to the use of new retarding agents in the dye baths with the cationic dyes.

It has been found that the use in the dye baths of products resulting from the cationization of polyamide resins having free hydrogen amines in the chain by salts of the type: halogenated epoxy propyltrialkyl ammonium corresponding to generic Formula I hereafter, permitted reduction of the velocity of taking up of the cationic dyes into the polyacrylonitrile fiber and to obtain thereby a good uniformity of the dyed material.

The salts of epoxy propyl trialkyl ammonium which serve to cationize the polyamide resins have the following formula:

### FORMULA I



in which R', R'' and R''' are alkyl radicals, identical or different, having one to three carbon atoms;

X represents groups such as the halide (Cl<sup>-</sup>), nitrate (NO<sub>3</sub><sup>-</sup>), sulphate (SO<sub>4</sub><sup>2-</sup>), etc.

Suitable polyamide resins for the preparation of the products used according to the present invention are the polyamides derived from polymeric fatty acids and polyalkylenespolyamines.

The polyalkylenes-polyamines have a generic formula:

### FORMULA II



in which x is at least equal to one;

R is an alkylene radical having one to five carbon atoms, such as ethylene, propylene, butylene, etc.

These polyamines should in addition contain at least four atoms of reactive hydrogen per molecule as, for example, ethylene diamine (E.D.A.), diethylene triamine (D.E.T.A.), triethylene tetramine (T.E.T.A.), etc.

The composition of the quaternized polyamino amide compounds which are known and used according to the present invention can be schematically represented by the following generic formula:

### FORMULA III



in which n is a number between one to twelve.

The quantities of cationic polyamide resin added to the dye bath for the polyacrylonitrile fibers to obtain the desired retarding effect are variable between large limits. It has been established, however, that a particularly suitable amount of the resin expressed as dry material is between 0.2 and 5 per weight of the fabric to be dyed.

The following examples which are given in an illustrative manner only, show how the invention can be put into practice. Examples 1-4 illustrate the qualities of uniformity of dyeing given in the presence of the cationic resins whereas Examples 5 and 6 show the equalizing effect of these resins in the dyeing, by migration of cationic dyes from a sample already dyed to a white sample.

### EXAMPLE 1

A sample of polyacrylonitrile fabric was introduced into an aqueous solution at 60°C containing 0.5% of blue dye, "C.I. (Color Index) basic blue 54," 4% of acetic acid (40%) and 0.5% of quaternized polyamino amide, the percentages given being calculated with respect to the weight of the fiber to be dyed. The proportion of dyeing bath was from one to twenty (that is, 20 ml of bath per 1 g. of material to be dyed).

The temperature was brought in 30 minutes to 100°C, then the dyeing was maintained at this temperature for an hour. After this period, the bath was practically exhausted. The sample was then subjected to a rinsing and then a drying.

There was obtained a blue shade having very good uniformity.

The polyamino amide utilized in the example was obtained by condensation of a fatty diacid (EMPOL 1024) with ethylene diamine, followed by quaternization by the chloride of epoxypropyltrimethyl ammonium.

### EXAMPLE 2

A sample of polyacrylonitrile fabric was introduced into an aqueous solution at 60°C containing 1% of violet dye, "C.I. (Color Index) basic violet 22," 4% of acetic acid (40%) and 1% of quaternized polyamino

amide, the percentages being calculated with respect to the weight of the fabric. The proportion of the bath was 1 to 20.

The conditions of dyeing were identical to those of Example 1, and there was obtained a violet color having an excellent uniformity.

The polyamino amide utilized was identical to that used in Example 1.

#### EXAMPLE 3

A sample of polyacrylonitrile fabric was dyed with the dye and under the same conditions as Example 1.

The polyamino amide was obtained by condensation of a fatty acid (EMPOL 1024) with diethylene triamine, then quaternized by the chloride of epoxypropyl trimethyl ammonium.

There is obtained a blue shade having perfect uniformity.

#### EXAMPLE 4

A sample of polyacrylonitrile fabric was dyed utilizing the dye and under the identical conditions as in Example 1.

The polyamino amide utilized was obtained by condensation of a fatty acid (EMPOL 1024) with triethylene tetramine, followed by quaternization by the chloride of epoxypropyl trimethyl ammonium.

There was obtained a blue color having good uniformity.

#### EXAMPLE 5

A sample of polyacrylonitrile fabric was dyed, for the first time, under the same conditions and with the same products as in Example 1.

After rinsing and drying, the blue sample of fabric was introduced simultaneously with a white sample of the same material of the same weight into an aqueous bath free of dye containing 4% of acetic acid (40%), 10% of NaCl and 4% of the quaternized polyamide of Example 1, the percentages being calculated in parts with respect to the bath. The proportion of bath was one to ten.

After treatment for 1 hour at 100°C followed by rinsing and drying of the samples, it was discovered that the initially white sample had taken on an intense blue coloration whereas in a comparative test effected under the same conditions but in the absence of the quaternized polyamide in the bath, it was found that the white sample had taken on a bluish tint, the color being very light and less sustained than that of the sample treated in the presence of the equalizer adjuvant of the present invention.

#### EXAMPLE 6

A sample of polyacrylonitrile fabric was dyed under the conditions of Example 1 except that the fabric was found to have numerous spots after dyeing, for example, caused by a poor rinsing.

The color was treated exactly as in Example 5 in a bath free of dye and containing the quaternized polyamide simultaneously with a white sample.

It was found that both the blue and the white samples

treated had taken on a beautiful uniform blue color, demonstrating a perfect migration and equalization of the initial dye.

It will be obvious to those skilled in the art that various changes may be made without departing from the scope of the invention and the invention is not to be considered limited to what is described in the specification.

What is claimed is:

- 10 1. A process for dyeing polyacrylonitrile fabrics in an aqueous bath containing a cationic colorant comprising adding to the bath as a retarding and equalization of dyeing agent, a quaternized polyamino amide obtained by the condensation of a fatty diacid with a polyamide having at least four reactive hydrogen atoms per molecule having the formula



in which  $x$  is at least equal to 1 and  $\text{R}$  is an alkylene radical containing one to five carbon atoms, the polyamino amide then being quaternized by a salt of epoxy propyl trialkyl ammonium of the formula



in which  $\text{R}'$ ,  $\text{R}''$  and  $\text{R}'''$  are alkyl radicals, identical or different, having one to three carbon atoms, and  $\text{X}$  is a radical selected from the group consisting of  $\text{Cl}^-$ ,  $\text{NO}_3^-$  and  $\text{SO}_4^{2-}$ .

- 25 2. A process according to claim 1 wherein the proportion of the quaternized polyamino amide added to the dye bath is between 0.2 and 5% per weight of the fabric to be dyed based on the dry material.

- 30 3. An aqueous dyeing bath for polyacrylonitrile fabrics comprising a cationic dye, and as a retarding and equalization of dyeing agent, a quaternized polyamino amide obtained by the condensation of a fatty diacid with a polyamine having at least four reactive hydrogen atoms per molecule having the formula



35 in which  $x$  is at least equal to 1 and  $\text{R}$  is an alkylene radical containing one to five carbon atoms, the polyamino amide then being quaternized by a salt of epoxy propyl trialkyl ammonium of the formula



40 45 55 in which  $\text{R}'$ ,  $\text{R}''$  and  $\text{R}'''$  are alkyl radicals, identical or different, having one to three carbon atoms, and  $\text{X}$  is a radical selected from the group consisting of  $\text{Cl}^-$ ,  $\text{NO}_3^-$  and  $\text{SO}_4^{2-}$ .

- 50 5. An aqueous dyeing bath according to claim 3 wherein the proportion of the quaternized polyamino amide in the dye bath is between 0.2 and 5% per weight of the fabric to be dyed based on the dry material.

\* \* \* \* \*